

## UNITED STATES PATENT OFFICE

2,115,341

## LUBRICATING OIL

Louis A. Mikeska and Luther B. Turner, Elizabeth, N. J., assignors to Standard Oil Development Company, a corporation of Delaware

No Drawing. Application June 22, 1934,  
Serial No. 731,991

## 16 Claims.

(Cl. 87—9)

The present invention relates to an improved lubricating composition and more particularly to an oil for the lubrication of automotive engines and other purposes. The invention will be fully understood from the following description.

It has been known and appreciated for some time that hydrocarbon oils could be improved in respect to their lubricating properties by the addition of relatively small amounts of materials which increase their oiliness. Various materials have been suggested but most of these have certain objections, for example, either that they are excessively corrosive, increase the carbon forming tendency of the oil or have an excessive oxidation rate. In the present application, which is a continuation in part of an earlier case, Serial No. 687,311, filed August 29, 1933, are disclosed a class of substances which are satisfactory for the present purposes in a very high degree.

The addition agents disclosed in the present case comprise the class of "acetylated" hydroxy acid compounds, by which is included the acids themselves, their esters and glycerides. Most of the acids, esters and glycerides are not miscible with mineral oils before acetylation but after such treatment they become in most cases miscible in all proportions.

The word "acetylation" as used in the present specification is intended to have a broader significance than the mere treatment with acetic acid or strictly acetylating materials but is intended to cover broadly the type of reaction whether the acid used be acetic or other low molecular weight acids, particularly those containing from 1 to 5 carbon atoms, among which formic, propionic, butyric and valeric may be mentioned, although it would be understood that unsaturated acids may also be used.

The materials which may be acetylated, as indicated above, include the hydroxy acids, esters and glycerides. The most important single substance is castor oil which is primarily the glyceryl ester of ricinoleic acid. Castor oil may be used as such or it may be subjected to hydrogenation in order to saturate the double bond. Among the acids which may be used may be mentioned the saturated hydroxy acids such as sabinic, juniperic and cocceric, which are merely mentioned as examples, but also the corresponding acids of the unsaturated or ricinoleic series, may also be used,

such as ricinoleic itself, isoricinoleic and ricinellidic. It will be understood furthermore, that the di-hydroxy or poly-hydroxy acids may also be used in which one or more of the hydroxyl groups are acetylated. Poly-basic acids can also be employed. Besides castor oil the glyceryl esters of all of the various acids of the classes mentioned above may be employed, and not only the glyceryl but glycol and mono-basic esters are also contemplated, especially the lower aliphatic alkyl esters prepared from alcohols containing from 1 to 5 carbon atoms. Hydroxy acids may, of course, be obtained from the oxidation product of paraffin wax, and such hydroxy acids may be either used as such in admixture with other constituents produced during the oxidation or they may be segregated in a known manner and used after acetylation. It will be understood that these acids may be used in a free state or they may be esterified with mono- or poly-basic alcohols.

The "acetylation", as indicated before, refers not only to the treatment with acetic acid or its equivalents but also to other low molecular weight acids. For some reason which is at present obscure the reaction products prepared by different acetylation methods are not equally good for present purposes. In general it has been found that the products produced by the acetylation with acid chlorides are more desirable than those prepared in any other manner. Oils containing relatively small amounts of a product prepared in this manner are capable of carrying heavier loads with less friction than similar compositions containing the products prepared by acetylation with acid anhydrides or with the acids themselves. As stated above, the reason for this is not fully understood but the superiority of the products prepared by acetylation with the acid chlorides is so substantial that these products are greatly preferred.

The acetylation may be conducted with acetic anhydrides or other acid anhydrides. The product of this reaction is found to be quite erratic in its load carrying or oiliness behavior. In a few instances the oily material has been very good but in most cases it is decidedly inferior to the product produced by acetylation with acetyl chloride. However, it has been found that a heat treatment or digestion at an elevated temperature, for example, from 200° C. to 400° C. which is well below

the decomposition point of the product, greatly enhances and stabilizes the oiliness properties of this product. The digestion may be accomplished under pressure in air or inert atmosphere, if desired. The time for such treatment is quite short but, of course, depends on temperature. The higher the temperature the shorter will be the time. It is often sufficient merely to distill over 10 to 20% of the reaction product in order to stabilize and greatly improve the undistilled fractions. In many instances there is a small acidity developed during the digestion step and before use of the product the acid should be removed, for example by neutralization or esterification 15 with a small amount of alcohol.

The material produced by direct acetylation with the organic acid, using sulphuric or some other strong dehydrating agent in the known manner, is also decidedly inferior to the product 20 produced in the preferred method using the acid chloride. The inferiority shows itself as indicated above, in lower load bearing capacity and a greater friction. This material can also be considerably improved by the heat treatment outlined in the previous paragraph.

The glyceryl esters of hydroxy acids, particularly castor oil, are the preferred raw materials for this process, and as has been indicated before, the preferred method is the acetylation by means 30 of an acid chloride which yields a product of high oiliness value giving low friction and which can be readily reproduced. It has been found that this product can be somewhat further improved by hydrogenation which saturates the double 35 bond. Such hydrogenation may be carried out with catalysts of the type of nickel, or others which are well known, and at temperatures of the order of from room temperature to 250° C. or higher, with a hydrogen pressure adjusted to 40 the activity of the catalyst so as to effect a saturation of the unsaturated bonds. The heat treatment mentioned above is not ordinarily necessary with the product produced by means of acetyl chloride or other acid chloride, but when the 45 product is produced by the other methods mentioned above such heat treatment is highly desirable and may be accomplished simultaneously with the hydrogenation.

The amount of the acetylated compounds to be 50 used depends to some extent on the particular material used, but in general only relatively small amounts are required, for example, as little as  $\frac{1}{2}$  of 1% frequently is sufficient to greatly increase the oiliness of a hydrocarbon lubricant, 55 but usually from 2 to 3 or up to 5 or 6% may be desired. The hydrogenation treatment improves not only the lubricating value of the compounds but also increases their stability to carbon deposition, and permits a somewhat larger amount to be used without excessive formation of carbon.

It has been found that the addition of these oiliness compounds ordinarily increases the oxidation rate of the lubricating oil employed. If the amount used does not exceed 5%, however, the 60 oxidation rate is not sufficiently increased to be objectionable in ordinary cases, but if larger amounts are used this may be objectionable. In any case the oxidation rate may be corrected by the addition of oxidation inhibitors which form a 65 large class of known compounds. Among these may be generally mentioned hydroxy or amino aromatics such as the naphthol and naphthyl amines, also thio phenolic aromatics such as the thio-naphthols, organic polysulphides, thio-ethers and di-sulphides, especially those containing aro-

matic groups, and also metallo organic compounds. Of these latter the lead, tin, mercury and bismuth aryl compounds are the most desirable although alkyl compounds are also useful.

The following examples are produced to illustrate the properties of the present compounds and the effect of the method of production:

(1) A sample of castor oil was acetylated by treatment with acetyl chloride in the well-known manner. Two percent of the product was then added to a highly refined petroleum lubricating oil S. A. E. grade 20. This compounded oil and a blank sample which contained none of the acetylated castor oil were then subjected to a test on the Mougey machine which has been described in 15 National Petroleum News vol. 23, #45. In these tests a steel pin and an aluminum bushing were used with the following results:

|                                                            | Weight carried | Final friction | 20 |
|------------------------------------------------------------|----------------|----------------|----|
| Oil.....                                                   |                |                |    |
| Same containing 2% acetylated castor oil (acetyl chloride) | 17             | Failure        |    |
|                                                            | 25             | 24             | 25 |

Each weight amounts to 1000 pounds per square inch load and the friction is given in pound feet.

(2) A product produced according to the method of Example 1 was carefully hydrogenated using a nickel catalyst, a pressure of one atmosphere, and a temperature of 25° C. Two percent of this material was added to the same oil used in Example 1 and on the Mougey machine the compound carried the full 25 weights with a maximum friction of 15.

(3) Six samples of acetylated castor oil were acetylated using acetic anhydride. In each case the oil was prepared in the same manner and with the same care. Two percent of each of the compounds were then added to the same oil and were subjected to the Mougey test with the following results. One sample was excellent and carried the full 25 weights with a final friction of 17. Two samples were fair, carrying full 25 weights with a friction ranging from 32 to 35. Three samples were quite inferior, causing a failure at from 23 to 25 weights with undesirably high frictional values.

(4) One of the poor samples of the acetylated mixture used in the previous example was carefully distilled, taking off approximately 15%. This product carried the full 25 weights with a final friction of 17.

(5) Four samples of castor oil were acetylated using a mixture of acetic and sulphuric acid. When used in the oil in proportion of 2% these samples carried from 24 to 25 weights with frictions from 60 to 95. Subjecting the above samples to heat treatment at a temperature of 300 to 340° C. for  $\frac{3}{4}$  hour improved the quality of the agents so that on the average they were able to carry 25 weights with a final friction of 10 to 17.

(6) A sample of castor oil was carefully hydrogenated and afterwards acetylated using a mixture of sulphuric and acetic acids. When used in proportion of about 2% it carried the full 25 weights on the Mougey machine with a final friction of 37.

(7) Two new automobiles, one a Ford and the second a Chevrolet, were "run in" on an oil containing 2% of the acetylated castor oil prepared by the acetyl chloride method. These cars were run for 1100 and 1600 miles at an average speed of 35 to 45 miles per hour, and at the end of the 75

period were found to be in excellent condition.

(8) Two percent and 5% respectively of acetylated castor oil were added to a well refined lubricating oil S. A. E. 20. The original blank and the two blended samples were then subjected to Sligh and oxidation tests with the following results:

|                                    | Sligh 24-hour | Oxidation rate |
|------------------------------------|---------------|----------------|
| 10 Blank sample                    | 19.1, 16.6    | 226            |
| Same plus 2% acetylated castor oil | 17.4          | 269            |
| Same plus 5% acetylated castor oil | 16.8          | 343            |

15

The Sligh test was conducted according to the ordinary or standard procedure with the exception that the heating period was for 24 hours. The oxidation rate is obtained by passing air continuously in a circuit bubbling through a 10 c. c. sample of the oil. After 15 minutes the amount of oxygen consumed is determined by difference as c. c. of oxygen consumed per 10 c. c. oil sample. By the use of suitable oxidation inhibitors, or combinations thereof, such as alpha naphthol amine, alpha thio-naphthol and lead tetraphenyl, hydroquinone, the oxidation rate of the above samples may be brought down in the range from about 200 to about 15 c. c. of oxygen absorbed per 10 c. c. of oil per 15 minutes.

The present invention is not to be limited to any particular oiliness compound known to any particular method of acetylation but only to the following claims in which it is desired to claim all novelty inherent in the invention.

We claim:

1. Lubricating composition comprising a viscous hydrocarbon oil containing from  $\frac{1}{2}$  to 5% of a product obtained by esterifying at least part 40 of the OH groups of a hydroxy acid compound of a long chain fatty acid with a low molecular weight ester-forming aliphatic reagent containing the group



45 and selected from the group consisting of acids, anhydrides and acid halides.

2. A composition according to claim 1 in which the esterified product is prepared by the action 50 of an acid halide on a hydroxy acid compound.

3. A composition according to claim 1 in which the esterified product is prepared by the action of an acid chloride on a hydroxy acid compound.

55 4. A composition of matter according to claim 1 in which the esterified product is produced by the action of an acid chloride on castor oil.

5. Composition of matter according to claim 1 in which the esterified product is produced by the 60 action of an acid chloride on castor oil and the final product subjected to hydrogenation.

6. Composition according to claim 1 in which the esterified product is prepared by the action of an acid anhydride on the hydroxy acid compound.

65 7. Composition according to claim 1 in which the esterified product is prepared by the action of acetic anhydride on a hydroxy acid compound,

and this product is subjected to heat treatment at an elevated temperature whereby its lubricating properties are enhanced.

8. Composition according to claim 1 in which the esterified product is prepared by the action 5 of an acid anhydride on castor oil and the product is subjected to heat treatment to enhance its lubricating qualities.

9. Composition according to claim 1 in which the esterified product is prepared by the action of 10 acetic anhydride on castor oil and the product is then subjected to hydrogenation.

10. Composition according to claim 1 in which the esterified product is produced by the action 15 of an organic acid on the hydroxy acid compound in the presence of a dehydrating agent.

11. Composition according to claim 1 in which the esterified product is prepared by the action of an organic acid with from 1 to 5 carbon atoms 20 on the hydroxy acid compound in the presence of sulphuric acid, and the product further subjected to heat treatment whereby its lubricating qualities are enhanced.

12. Composition according to claim 1 in which the esterified product is prepared by the action 25 of an organic acid with from 1 to 5 carbon atoms on the hydroxy acid compound in the presence of castor oil, and the product further subjected to hydrogenation whereby its lubricating qualities are improved.

30 13. Composition according to claim 1 in which the esterified product is subjected to heat treatment at elevated temperature whereby its lubricating properties are enhanced.

14. Composition according to claim 1 in which the esterified product is prepared by the action 35 of the said acid halide on the said hydroxy acid compound and the esterified product is subjected to hydrogenation.

15. Composition according to claim 1 in which the esterified product is prepared by the action 40 of the said organic acid on the said hydroxy acid compound and the esterified product is subjected to heat treatment whereby its lubricating qualities are enhanced.

45 16. Lubricating oil composition comprising a viscous hydrocarbon oil containing a small proportion of an ester having the formula,



50

55

55

in said formula represents the alkoxy group of a 60 hydroxy acid compound, having at least one OH group, of a long-chain fatty acid compound, R and R' represent alkyl groups, X represents H or an alkyl group of one to five carbon atoms, and R'' represents a low molecular weight alkyl group 65 of one to about four carbon atoms.

LOUIS A. MIKESKA.  
LUTHER B. TURNER.